

April 21, 1970

R. F. TAMM ET AL

3,507,655

PLASTIC MARKING PROCESS

Filed July 24, 1967



BY

INVENTORS  
RICHARD F. TAMM  
JAMES M. THRONE  
*Paul Sheppard*  
ATT'Y.

1

3,507,655

## PLASTIC MARKING PROCESS

Richard F. Tamm, Elmhurst, and James M. Throne, Country Club Hills, Ill., assignors to Continental Can Company, Inc., New York, N.Y., a corporation of New York

Filed July 24, 1967, Ser. No. 655,387

Int. Cl. G03c 1/92

U.S. CL. 96—45.1

8 Claims

## ABSTRACT OF THE DISCLOSURE

A method for providing a code marking invisible in normal light on a plastic substrate exhibiting fluorescent properties wherein a source of intense optical radiation is impinged on the substrate through a stencil bearing the desired marking pattern, the radiation causing a change in the fluorescence of the substrate in the radiated area. The resultant marking is invisible in ordinary light, but visible under ultra-violet illumination.

## BACKGROUND OF THE INVENTION

## Field of the invention

The present invention relates to the marking of plastic substrates and more particularly relates to a means for marking a plastic material having fluorescent properties using optical radiation.

## The prior art

In the packaging of materials in plastic containers, it is frequently desired to apply to the surface of the container some designation or code number which serves to indicate the source of the particular lot of material being packaged, the time or date when the particular material was packaged, or other information. Many times it is also desirable that the code or marking be invisible, as for example, where it is desired to follow the manufacturing history of the container without defacing the container.

Generally, the code marking is embossed on the plastic container surface by metal dies which is a time-consuming and expensive procedure.

## SUMMARY OF THE INVENTION

The present invention provides a means of producing on a plastic substrate having fluorescent properties a marking invisible in ordinary light but which can be read when subjected to the proper selective light or energy wavelength wherein an opaque stencil having an aperture pattern corresponding to the desired marking is placed between the substrate to be marked and a source of optical radiation, the substrate being so positioned that the aperture pattern of the stencil is in registration with the portion of the substrate on which it is desired to produce the invisible marking, whereupon the source of optical radiation is impinged on the substrate through the apertures of the stencil, the source of optical radiation transmitting sufficient energy to the substrate surface to cause a change in the fluorescence of the substrate exposed to the source of optical radiation.

## DESCRIPTION OF THE DRAWING

In the accompanying figure is illustrated a schematic representation of an apparatus for projecting a source of optical radiation through an opaque stencil to produce a marking invisible in natural light but visible in ultraviolet light on the surface of a fluorescent plastic substrate.

Referring to the figure, a plastic substrate 10 which exhibits fluorescence in filtered ultraviolet light is transportable from supply roll 11 past a marking station indicated

2

by the arrow 12 to be taken up on take-up roll 13. The fluorescent plastic substrate 10 is sensitive to the optical radiation from a source 14 which is directed thereon through stencil 15 having aperture pattern 15A corresponding to the marking which is desired to be printed on the surface of the substrate 10.

The stencil 15 is placed adjacent to the moving substrate 10 in a position at which the aperture pattern 15A is in registration with the portion of the substrate 10 at which it is desired to mark the substrate as it passes through the marking station 12.

The source of optical radiation 14 is illustrated diagrammatically as one or more lamps 16 with series current distribution connections thereof which are located in close proximity to the moving substrate 10. The lamps 16 are housed in an opaque base 17 having an opening 18 and a reflector 19 to reflect light rays from which the optical radiation is projected to the stencil 15. The lamps 16 are electrically connected to a power supply which furnishes high voltage direct current for energizing the lamps.

The lamps 16 will be understood to be such as will radiate any suitable form of optical radiation which will furnish an amount of energy which is effective to cause a change in the fluorescence of the fluorescent plastic substrate.

For example, the lamp 16 can be formed from a tube or envelope made of fused quartz which contains an inert gas such as xenon or krypton under reduced pressure. Such lamps emit a high energy continuous spectrum light when energized.

The wavelengths of the light emitted by the lamp 16 are both in the infra-red and ultra-violet range and include as well, wavelengths of some or all the light in the intermediate or visible spectrum. Ultraviolet light having wavelengths ranging from 4000 angstroms, for example, to a lower limit of 1800 angstroms, which is the limit for the transmission of ultra-violet light through quartz, is particularly desirable for the purpose of the present invention and a light source of the type described is particularly efficient in producing an abundance of light between these wavelengths.

The source of optical radiation 14 may be operated continuously with exposure controlled by means of a suitable shutter or of the instantaneous discharge or flash type which may be operated intermittently as required for exposure.

## PREFERRED EMBODIMENTS

The areas of the plastic substrate marked by exposure to the optical radiation are invisible in ordinary light but exhibit a fluorescence different from the fluorescent color of the unexposed areas of the fluorescent substrate in accordance with the pattern of the apertures in the stencil when viewed in ultraviolet light. The visual impact of the marking results from the contrast developed between the initial background and the changed fluorescent areas and can be readily identified. The change in fluorescence in the radiated area can be either significantly more or less fluorescence or fluorescence of a significantly different color or wave length.

There are many polymeric materials known to the art which exhibit fluorescence in filtered ultraviolet light. For example, when viewed in ultraviolet light, synthetic resins such as phenol-formaldehyde resins have an intense blue-violet fluorescence, thiourea-formaldehyde resins have a bluish-white fluorescence, cellulose-acetate has a faint bluish-white fluorescence, cellulose-nitrate has a yellow-brown fluorescence, polyacrylic acid has an intense blue fluorescence, polybutadiene has a bright violet fluorescence, polystyrene has a blue-violet fluorescence, chlorinated rubber has a pale light blue fluorescence, polyvinylacetate has a white-blue fluorescence, polyvinylalco-



At 28% conversion, a copolymer containing 28.6% glycidyl ester and 40.2% chlorine was obtained. The intrinsic viscosity of the copolymer was 0.187 poise at 30° C. Forty grams of the copolymer were dissolved in a mixture of 51 grams of toluene and 9 grams of isopropanol along with one gram of Versamide 125 which is a condensation product of a polymerized fat and a poly-amine of the type described in U.S. Patent 2,379,413.

The coating composition was applied to a tinplate surface and baked 8 minutes at 325° F. Cured coated samples were marked in accordance with the procedure of Example I over the range of 2.5 to 4.0 kilovolts. The amount of energy transmitted to the substrate over this range was 1.5 to 3.5 joules/cm.<sup>2</sup>.

None of the samples exhibited a print visible in normal light but all exhibited a clearly readable coaded image under ultraviolet light. At 3200-4000 AU, the coded image was a non-fluorescent marking on an overall fluorescent background. At 3.5 kilovolts, i.e., at 3.0 joules/cm.<sup>2</sup> of substrate surface, image visibility under ultraviolet light was excellent, as evidenced by extinction voltage of 75 volts.

The markings on the samples were found to be extremely stable, as there was no sognificant alteration of the coded image when the flashed samples were exposed to water at 160° F. for 20 minutes or exposed to room illumination, that is, a cool, white fluorescent lamp and stored in the dark for over 6 months.

#### Example V

A film, about 4 mils thick, which was cast from a copolymer containing 86% vinyl chloride, 13% vinyl acetate, and 1% maleic acid, was irradiated at 4.0 kilovolts, 1250 joules, following the procedure of Example I using a reflective metal surface to backup the film. The amount of energy transmitted to the substrate was 3.5 joules/cm.<sup>2</sup>. An examination of both sides of the films indicated that the marking could be read from either side of the film.

What is claimed is:

1. A process for producing a marking invisible in natural light but visible in ultraviolet light on a plastic substrate exhibiting fluorescent properties in filtered ultraviolet light which comprises the steps of positioning an

opaque stencil having an aperture pattern corresponding to the desired marking between the substrate to be marked and a source of optical radiation so that the aperture pattern is in registration with the portion of the substrate on which it is desired to produce the marking, impinging the source of optical radiation on the substrate through the apertures of the stencil, the source of optical radiation transmitting sufficient energy to the substrate surface to cause a change in the fluorescence of the substrate in the areas exposed to the source of optical radiation, the change in fluorescence being discernible only in ultraviolet light.

2. The process of claim 1 wherein the plastic substrate is comprised of an epoxy resin.

3. The process of claim 1 wherein the substrate is a copolymer containing vinyl chloride.

4. The process of claim 1 wherein the substrate is a vinyl chloride/vinyl acetate copolymer.

5. The process of claim 1 wherein the substrate is a vinyl chloride/vinyl acetate/maleic acid terpolymer.

6. The proces of Example I wherein the source of optical radiation is a flash lamp which emits a high-energy, continuous spectrum light.

7. The process of Example 1 wherein the source of optical radiation is a xenon-filled quartz tube.

8. The process of claim 1 wherein the source of optical radiation transmits to the substrate an amount of energy in the range of about 1 to about 6 joules/cm.<sup>2</sup> of substrate surface.

#### References Cited

##### UNITED STATES PATENTS

3,330,680 7/1967 Haas ----- 96—45.1

##### OTHER REFERENCES

35 Simonds et al., Handbook of Plastics, Table 107, (1943).

40 SAMUEL H. BLECH, Primary Examiner

R. B. TURER, Assistant Examiner

##### U.S. Cl. X.R.

117—33.5; 161—33, 164, 412; 204—159.2, 159.14